

## UNITED STATES PATENT OFFICE

2,473,166

## PROCESS FOR THE PRODUCTION OF PHOTOGRAPHIC IMAGES BY COLOR DEVELOPMENT

Philipbert Raymond Merckx, Mortsel-Antwerp, Belgium, assignor to Gevaert Photo-Producten N. V., Mortsel-Antwerp, Belgium, a company of Belgium

No Drawing. Application February 26, 1948, Serial No. 11,324. In Belgium August 3, 1945

Section 1, Public Law 690, August 8, 1946  
Patent expires August 3, 1965

8 Claims. (Cl. 95—6)

1

This invention relates to the production of photographic images by color development, and more particularly to a new group of color couplers.

It is known in the art of color development to use color couplers which correspond to the following general formula



wherein

Y is an electro-negative group,

R is amino, substituted by an aryl- or heterocyclic group.

It is further known to use as color couplers, 1-2-4-oxadiazols of the following general formula



wherein

X is an electro-negative organic radical, for instance CN, alkyl-CO, aryl-CO,

Y is an organic radical, hydrogen.

It is an object of my invention to provide a new process for developing reducible silver salt images.

It is also an object of my invention to provide a process for the production of colored photographic images.

Another object of my invention is to provide a new color developer.

Still another object of my invention is to provide new light-sensitive silver halide emulsions.

A further object of my invention is to provide a colored photographic image.

Further objects will appear from the following description.

These objects are accomplished by developing a reducible silver salt image with an aromatic amino developing agent in the presence of a compound corresponding to the following general formula



wherein

Z is O or S.

Y is hydrogen, an aliphatic-, homo- or heterocyclic group either substituted or not.

The reactive methylene group may also be substituted by atoms or groups which, on developing, easily split-off, such as for instance bromo.

It is sufficient that on development, a com-

2

ound corresponding to the last mentioned formula is present. Therefore, it is sufficient to add to the photographic material or to the developer at any step in the manufacture or in the processing of the photographic material, a substance capable of forming before or during development said compound corresponding to the said formula.

Compounds according to my invention are:

[2-p-nitrophenyl-1,3,4-oxadiazolyl(5)]acetonitrile



1,3,4-oxadiazolyl-2,5-di-acetonitrile



[2-p-tolyl-1,3,4-thiodiazolyl(5)]acetonitrile



25 These nitriles may be prepared for instance from NN'-substituted hydrazides having at least one CN—CH<sub>2</sub>—CO group. For instance for the preparation of [2-p-nitrophenyl-1,3,4-oxadiazolyl (5)] acetonitrile, 15.3 g. of



are mixed with 15 cm.<sup>3</sup> phosphoroxy-chloride. This mixture is heated for two hours on an oil bath at 130–140° C. The thick oil obtained is poured upon 250 g. finely cracked ice.

The brown precipitate formed is purified by boiling with alcohol.

It is noteworthy that, depending on the kind and substitution of the group Y, these new color couplers yield the widest different tones. Also the substitution of the oxygen atom in the nucleus by S enables the shifting of the absorption maximum.

45 In practicing my invention, the new color couplers may either directly be added to the photographic colloid layer, either before or after coating so that the colored image is formed by developing with an aromatic developer, or the colored image may be obtained by developing the photographic image with an aromatic developer which contains one of the above-defined color couplers.

The colloid layer to which the color coupler is added, may be a light-sensitive silver halide

emulsion layer or a non-light-sensitive layer adjacent thereto or separated therefrom by a water permeable colloid layer. When the color coupler is added to a colloid layer, it is desirable that the group Y contain a group rendering the coupler fast to diffusion.

A developing bath for obtaining color images according to my invention is the following:

A  
N,N-diethyl-paraphenylenediamine

hydrochloride ..... grams 5  
Sodium sulphite (cryst.) ..... do 10  
Sodium carbonate (cryst.) ..... do 100  
Sodium hydroxide ..... do 1  
Water ..... cm.<sup>3</sup> 1000

B



Acetone ..... cm.<sup>3</sup> 30

Before using, B is added to A.

My invention may be used for obtaining colored photographic images upon plates, paper or film, coated with a light-sensitive silver halide emulsion. The color developing process may be used for developing photographic material with one or more light-sensitive layers coated on one side or on both sides of the support.

The silver image, formed during the development, can easily be removed by treatment in a bleach-bath. The bleach-bath used, however, is not allowed to exert a noxious influence upon the colored image. A bleach-bath of potassium ferricyanide and sodium thiosulphate, removes the silver without damaging the color image.

I claim:

1. Process for the production of photographic color images by color development, which comprises developing a reducible silver salt image with a primary aromatic amino developing agent in the presence of a compound of the following general formula:



wherein

Z is a member selected from the group consisting of O and S,

Y is a member selected from the group consisting of aliphatic-, homo- and heterocyclic groups.

2. Process for the production of photographic color images by color development, which comprises developing a reducible silver salt image with a developer containing a primary aromatic amino developing agent and a compound of the following general formula:



wherein

Z is a member selected from the group consisting of O and S,

Y is a member selected from the group consisting of aliphatic-, homo- and heterocyclic groups.

3. Process for the production of photographic color images by color development, which comprises developing with a primary aromatic amino developing agent a reducible silver salt image in a light-sensitive silver salt emulsion containing a compound of the following general formula:



wherein

Z is a member selected from the group consisting of O and S,

Y is a member selected from the group consisting of aliphatic-, homo- and heterocyclic groups.

4. Color photographic developer containing a primary aromatic amino developing agent and a compound of the following general formula:



wherein

Z is a member selected from the group consisting of O and S,

Y is a member selected from the group consisting of aliphatic-, homo- and heterocyclic groups.

5. Color photographic developer containing a primary aromatic amino developing agent and 12-p-nitrophenyl-1,3,4-oxadiazolyl(5)acetonitrile.

6. Color photographic developer containing a primary aromatic amino developing agent and 1,3,4-oxadiazolyl-2,5-di-acetonitrile.

7. Color photographic developer containing a primary aromatic amino developing agent and 12-p-tolyl-1,3,4-thiodiazolyl(5)acetonitrile.

8. Light-sensitive silver halide emulsion containing a compound of the following general formula



wherein

Z is a member selected from the group consisting of O and S,

Y is a member selected from the group consisting of aliphatic-, homo- and heterocyclic groups.

PHILIBERT RAYMOND MERCKX.

REFERENCES CITED

60 The following references are of record in the file of this patent:

FOREIGN PATENTS

| Number     | Country | Date          |
|------------|---------|---------------|
| 65 836,144 | France  | Oct. 10, 1938 |